# EUROPEAN PATENT SPECIFICATION

(11) **EP 1 683 879 B1**
(45) Date of publication and mention of the grant of the patent: **25.11.2009**
(21) Application number: 06001442.0
(22) Date of filing: 24.01.2006
(51) Int. Cl.: C22B 34/36, B22F 1/00, B22F 1/02, C23F 11/00

(54) **Additives for suppressing tungsten leachability**
Zusatzmittel zum Unterdrücken der Auslaugung von Wolfram
Additifs pour supprimer le lessivage du tungstène

(30) Priority: 24.01.2005 US 593536 P; 09.01.2006 US 306705
(43) Date of publication of application: 26.07.2006
(73) Proprietor: OSRAM SYLVANIA INC., Danvers, MA 01923 (US)
(72) Inventor: Lunk, Hans-Joachim, Towanda, PA 18848 (US); Morgan, Ricky D., Milan, PA 18831 (US); Stevens, Henry J., Athens, PA 18810 (US)
(74) Representative: Grünecker, Kinkeldey, Stockmair & Schwanhäusser Anwaltssozietät

(56) References cited:
- EP-A- 0 279 454
- DE-C- 78 315
- US-A- 4 397 821
- US-A- 4 800 316
- US-A- 5 656 791
- US-A1- 2003 056 620
- PATENT ABSTRACTS OF JAPAN vol. 012, no. 108 (E-597), 7 April 1988 (1988-04-07) & JP 62 239622 A (HITACHI LTD), 20 October 1987 (1987-10-20)
- PATENT ABSTRACTS OF JAPAN vol. 2003, no. 11, 5 November 2003 (2003-11-05) & JP 2003 211144 A (KURITA WATER IND LTD), 29 July 2003 (2003-07-29)
- DATABASE WPI Section Ch, Week 197932 Derwent Publications Ltd., London, GB; Class M22, AN 1979-58665B XP002392236 & JP 54 080208 A (TOKYO SHIBAURA ELECTRIC CO) 26 June 1979 (1979-06-26)
- DATABASE WPI Section Ch, Week 198445 Derwent Publications Ltd., London, GB; Class M22, AN 1984-278420 XP002392237 & JP 59 170206 A (NIPPON TUNGSTEN KK) 26 September 1984 (1984-09-26)
- DATABASE WPI Section Ch, Week 198804 Derwent Publications Ltd., London, GB; Class L03, AN 1988-025617 XP002392238 & JP 62 286698 A (HOKKAI TUNGSTEN KOGYO KK) 12 December 1987 (1987-12-12)
- DATABASE WPI Section Ch, Week 200308 Derwent Publications Ltd., London, GB; Class M22, AN 2003-085298 XP002392244 & JP 2002 332505 A (NISHIDA T) 22 November 2002 (2002-11-22)
- DATABASE WPI Section Ch, Week 199402 Derwent Publications Ltd., London, GB; Class L02, AN 1994-012831 XP002392245 & JP 05 320943 A (SHOWA DENKO KK) 7 December 1993 (1993-12-07)

## Description

The use of tungsten powder or pressed tungsten powder compacts in pure or mixtures with other powders under natural conditions in the presence of water and oxygen (e.g., air or dissolved oxygen) leads to the formation of a water-soluble, tungsten-containing species. The first step of the reaction can be described as follows:

W + H₂O + 1.5 O₂ --> WO₄²⁻ + 2 H⁺.

The monotungstate ion, WO₄²⁻, reacts with H⁺, resulting in the formation of the soluble metatungstate anion [H₂W₁₂O₄₀]⁶⁻:

12 WO₄²⁻ + 18 H⁺ --> [H₂W₁₂O₄₀]⁶⁻ + 8 H₂O.

The formation of this polyoxometalate anion is detectable by its typical UV absorption maximum at 256 nm (molar extinction coefficient, ∈₂₅₆ = 3.8x10⁴ L(mol·cm)⁻¹).

JP-A-05-320943 discloses a metallizing paste for an aluminum nitride sintered compact containing tungsten powder and oxides of aluminum, silicon, yttrium, calcium and tungsten.

US-A-5656791 discloses a composition comprising a mixture of tungsten powder and a powdered metal binder, which may be lead.

JP-A-2002-332505 discloses a self lubricative sintered material obtained by sintering a mixed powder containing molybdenum disulfide powder, black lead powder, tungsten disulfide powder, tungsten powder, and ferrite stainless steel powder.

DE-C-78315 discloses a process for the preparation of a projectile, said process comprising the steps of mixing tungsten powder and a powder of a low melting metal or an alloy thereof, and heating the obtained mixture to the melting point of the low melting metal or metal alloy. Examples of the low melting metals and alloys thereof include bismuth, tin, lead, mercury, and alloys thereof.

It has been discovered that the leachability of tungsten in an aqueous medium may be suppressed by using a suitable additive that will cause an insoluble tungsten-containing compound to form under conditions which would normally cause leaching of the tungsten. As used wherein, insoluble means no significant solubility in the relevant aqueous medium under ambient conditions.

The present invention provides a method of suppressing the leachability of tungsten powder or tungsten powder compacts, said method comprising the steps of combining tungsten metal with a compound selected from lead oxide, lead nitrate, lead bromide, lead chloride, lead fluoride, lead sulfate, lead oxalate and calcium sulfate, contacting the combination with an aqueous medium, and forming an insoluble tungsten-containing compound.

The present invention further provides a powder mixture comprising a mixture of powdered tungsten metal and a powdered compound selected from lead oxide, lead nitrate, lead bromide, lead chloride, lead fluoride, lead sulfate, lead oxalate and calcium sulfate, wherein the amount of the compound is from 1 weight percent to 10 weight percent of the tungsten.

Moreover, the present invention provides a tungsten-containing article comprising tungsten metal and a compound selected from lead oxide, lead nitrate, lead bromide, lead chloride, lead fluoride, lead sulfate, lead oxalate and calcium sulfate, wherein the amount of the compound is from 1 weight percent to 10 weight percent of the tungsten.

Preferred embodiments of the present invention are set forth in the sub-claims.

More particularly, tungsten metal is combined with a specific metal oxide or metal salt that will form the insoluble tungsten-containing compound when the mixture is brought into contact with an aqueous medium, preferably having a pH from 4 to 9. The additive is present preferably in an amount from 1 weight percent (wt.%) to 10 weight percent of the tungsten, and, more preferably, from 1 wt.% to 2 wt.% of the tungsten.

The additive must be more soluble in the aqueous medium than the insoluble tungsten-containing compound to be formed. Possible additives include lead oxide, and calcium sulfate or lead nitrate. Preferably, the insoluble tungsten-containing compounds that are formed are tungstates, and, more preferably, lead tungstate (solubility at 25°C of 2.7x10⁻⁶ mol/L) or calcium tungstate (solubility at 25°C of 4.3x10⁻⁵mol/L).

In a preferred embodiment, the invention may be carried out by mixing powdered tungsten metal with a powdered form of the additive. A binder material may be also be added for facilitating the pressing of a tungsten-containing article. Or alternatively, it may be possible for some tungsten/additive powder mixtures to be pressed directly into the desired shape without an additional binder depending upon the mechanical strength needed for the pressed article.

For a better understanding of the present invention, together with other and further objects, advantages and capabilities thereof, reference is made to the following disclosure and appended claims.

Ten-gram amounts of a tungsten metal powder (particle size > 3 micrometers) were mixed separately with various amounts of lead oxide, and calcium sulfate, and added to 500-ml volumes of an aqueous buffer solution in 1-liter NALGENE© (PP) Erlenmeyer flasks. The buffer solution having a pH of 7.2 was prepared by dissolving 4.03 mg KCI, 50.6 mg CaSO₄·2H₂O, 123.2 mg MgSO₄·7H₂O, 96.0 mg NaHCO₃, and 209.3 mg of a noncomplexing tertiary amine, 3-(N-morpholino) propanesulfonic acid (MOPS) per liter of water. For a control, 10 g of tungsten metal powder alone was also placed in 500 ml of the aqueous buffer solution.

In another series of tests, 10-g amounts of tungsten metal powder were placed in 500-ml volumes of an unbuffered aqueous solution of lead nitrate (pH 4.4) in 1-liter NALGENE© (PP) Erlenmeyer flasks. In this case, the additive amount in Table 1 is given in terms of the molarity of the lead nitrate solution. Other lead salts that may be used based on their solubilities include lead bromide, lead chloride, lead fluoride, lead sulfate and lead oxalate.

The 1-liter flasks containing the samples were loosely covered with an aluminum foil and continuously shaken in a dark, thermostated room (72°F) with a LAB-LINE® Force orbital open air shaker, Model 4690, for a period of 28 days. Periodic 25-ml samples of the leachate solutions were taken and analyzed for pH, oxygen content, and tungsten content at 7, 14, 21, and 28 days. A constant oxygen concentration of 8.3 ± 0.2 mg/liter was observed for the entire testing period of 28 days.

The results of the leach tests are shown in Table I. Weight percentages of the additives are based on the amount of tungsten. As can be seen from the Control sample, the amount of tungsten in the leachate increases from 0.32% of the initial tungsten at 7 days to 0.78% at 28 days. In most cases, the leachability of tungsten is suppressed compared to the Control, and in many cases is zero (i.e., below the detection limit of 0.4 mg W/L). The addition of lead oxide showed a distinct improvement at levels of 2 wt.% or higher. At 1 wt.%, lead oxide had only a minor suppressing effect on tungsten's leachability. In some cases, e.g., 10 wt.% calcium sulfate, the amount of leached tungsten actually decreased over time indicating that the amount of additive entering solution increased as time progressed.

Table I: Effect of various additives on tungsten leachability (in % based on initial W amount)

| Sample | Additive | Additive Amount (wt.%) | Starting pH | %W 7-day | %W 14-day | %W 21-day | %W 28-day |
|---|---|---|---|---|---|---|---|
| W powder (control) | --- | --- | 7.2 | 0.32 | 0.49 | 0.65 | 0.78 |
| W powder | lead oxide | 1 | 7.2 | 0.28 | 0.47 | 0.59 | 0.68 |
| W powder | lead oxide | 2 | 7.2 | 0.00 | 0.004 | 0.16 | 0.21 |
| W powder | calcium sulfate | 1 | 7.2 | 0.28 | 0.25 | 0.21 | 0.24 |
| W powder | calcium sulfate | 10 | 7.2 | 0.14 | 0.06 | 0.04 | 0.03 |
| | | | | | | | |

| Sample | Additive | Additive Conc. | Starting pH | %W 7-day | %W 14-day | %W 21-day | %W 28-day |
|---|---|---|---|---|---|---|---|
| W powder | Pb(NO₃)₂ | 0.01 M | 4.4 | 0.00 | 0.00 | 0.00 | 0.00 |
| W powder | Pb(NO₃)₂ | 0.001 M | 4.4 | 0.00 | 0.00 | 0.00 | 0.00 |
| W powder | Pb(NO₃)₂ | 0.0005M | 4.4 | 0.00 | 0.00 | 0.00 | 0.04 |
| W powder | Pb(NO₃)₂ | 0.0001 M | 4.4 | 0.00 | 0.04 | 0.13 | 0.23 |

## Claims

1. A method of suppressing the leachability of tungsten powder or tungsten powder compacts, said method comprising the steps of combining tungsten metal with a compound selected from lead oxide, lead nitrate, lead bromide, lead chloride, lead fluoride, lead sulfate, lead oxalate and calcium sulfate, contacting the combination with an aqueous medium, and forming an insoluble tungsten-containing compound.

2. The method of claim 1, wherein the insoluble tungsten-containing compound is lead tungstate or calcium tungstate.

3. The method of claim 1, wherein the pH of the aqueous medium is from 4 to 9.

4. The method of claim 1, wherein the amount of the compound is from 1 weight percent to 10 weight percent of the tungsten.

5. The method of claim 4, wherein the amount of the compound is from 1 weight percent to 2 weight percent of the tungsten.

6. A powder mixture comprising a mixture of powdered tungsten metal and a powdered compound selected from lead oxide, lead nitrate, lead bromide, lead chloride, lead fluoride, lead sulfate, lead oxalate and calcium sulfate, wherein the amount of the compound is from 1 weight percent to 10 weight percent of the tungsten.

7. The powder mixture of claim 6, wherein the amount of the compound is from 1 weight percent to 2 weight percent of the tungsten.

8. A tungsten-containing article comprising tungsten metal and a compound selected from lead oxide, lead nitrate, lead bromide, lead chloride, lead fluoride, lead sulfate, lead oxalate and calcium sulfate, wherein the amount of the compound is from 1 weight percent to 10 weight percent of the tungsten.

9. The tungsten-containing article of claim 8, wherein the amount of the compound is from 1 weight percent to 2 weight percent of the tungsten.

## Patentansprüche

1. Verfahren zum Unterdrücken der Auslaugung von Wolframpulver oder Wolframpulverpresskörpern, wobei das Verfahren die Schritte umfasst:
Verbinden von Wolframmetall mit einer Verbindung gewählt aus Bleioxid, Bleinitrat, Bleibromid, Bleichlorid, Bleifluorid, Bleisulfat, Bleioxalat und Calciumsulfat, in Kontakt bringen der Kombination mit einem wässrigen Medium und Formen einer unlöslichen wolframhaltigen Verbindung.

2. Verfahren nach Anspruch 1, wobei die unlösliche wolframhaltige Verbindung Bleiwolframat oder Calciumwolframat ist.

3. Verfahren nach Anspruch 1, wobei der pH-Wert des wässrigen Mediums von 4 bis 9 beträgt.

4. Verfahren nach Anspruch 1 , wobei die Menge der Verbindung von 1 Gew.% bis 10 Gew.-% des Wolframs beträgt.

5. Verfahren nach Anspruch 4, wobei die Menge der Verbindung zwischen 1 Gew.-% bis 2 Gew.-% des Wolframs beträgt.

6. Pulvermischung umfassend eine Mischung aus pulverförmigen Wolframmetall und einer pulverförmigen Verbindung gewählt aus Bleioxid, Bleinitrat, Bleibromid, Bleichlorid, Bleisulfat, Bleioxalat und Calciumsulfat, wobei die Menge der Verbindung von 1 Gew.-% bis 10 Gew.-% des Wolframs beträgt.

7. Pulvermischung nach Anspruch 6, wobei die Menge der Verbindung von 1 Gew.-% bis 2 Gew.% des Wolframs beträgt.

8. Wolframhaltiger Gegenstand umfassend Wolframmetall und eine Verbindung gewählt aus Bleioxid, Bleinitrat, Bleibromid, Bleichlorid, Bleifluorid, Bleisulfat, Bleioxalat und Calciumsulfat, wobei die Menge der Verbindung von 1 Gew.-% bis 10 Gew.-% des Wolframs beträgt.

9. Wolframhaltiger Gegenstand nach Anspruch 8, wobei die Menge der Verbindung von 1 Gew.% bis 2 Gew.-% des Wolframs beträgt.

## Revendications

1. Procédé pour supprimer l'aptitude à la lixiviation de la poudre de tungstène ou de comprimés de poudre de tungstène, ledit procédé comprenant les étapes de combinaison du tungstène métallique avec un composé choisi parmi l'oxyde de plomb, le nitrate de plomb, le bromure de plomb, le chlorure de plomb, le fluorure de plomb, le sulfate de plomb, l'oxalate de plomb et le sulfate de calcium, de mise en contact de la combinaison avec un milieu aqueux, et la formation d'un composé contenant du tungstène, insoluble.

2. Procédé de la revendication 1, dans lequel le composé contenant du tungstène, insoluble, est le tungstate de plomb ou le tungstate de calcium.

3. Procédé de la revendication 1, dans lequel le pH du milieu aqueux est de 4 à 9.

4. Procédé de la revendication 1, dans lequel la quantité du composé est de 1 % en poids à 10 % en poids du tungstène.

5. Procédé de la revendication 4, dans lequel la quantité du composé est de 1 % en poids à 2 % en poids du tungstène.

6. Mélange pulvérulent comprenant un mélange de tungstène métallique en poudre et d'un composé en poudre choisi parmi l'oxyde de plomb, le nitrate de plomb, le bromure de plomb, le chlorure de plomb, le fluorure de plomb, le sulfate de plomb, l'oxalate de plomb et le sulfate de calcium, dans lequel la quantité du composé est de 1 % en poids à 10 % en poids du tungstène.

7. Mélange pulvérulent de la revendication 6, dans lequel la quantité du composé est de 1 % en poids à 2 % en poids du tungstène.

8. Objet contenant du tungstène comprenant du tungstène métallique et un composé choisi parmi l'oxyde de plomb, le nitrate de plomb, le bromure de plomb, le chlorure de plomb, le fluorure de plomb, le sulfate de plomb, l'oxalate de plomb et le sulfate de calcium, dans lequel la quantité du composé est de 1 % en poids à 10 % en poids du tungstène.

9. Objet contenant du tungstène de la revendication 8, dans lequel la quantité du composé est de 1 % en poids à 2 % en poids du tungstène.
